

Feb. 22, 1927.

1,618,612

R. TULL

TRANSFER AND METHOD OF MAKING THE SAME.

Filed June 28, 1926



By

Inventor  
Roger Tull

*Lyon & Lyon*

Attorneys

Patented Feb. 22, 1927.

1,618,612

# UNITED STATES PATENT OFFICE.

ROGER TULL, OF LOS ANGELES, CALIFORNIA, ASSIGNOR TO WESTERN LITHOGRAPH COMPANY, OF LOS ANGELES, CALIFORNIA, A CORPORATION OF CALIFORNIA.

## TRANSFER AND METHOD OF MAKING THE SAME.

Application filed June 28, 1926. Serial No. 119,039.

This invention relates to methods of making transfers, said transfers being more especially of a type comprising transfer paper provided with a coat or plurality of coats of paint

The invention also relates to the product that results from the practice of the new method.

The accompanying drawings illustrate the invention.

Figure 1 is a face view of a transfer constructed in accordance with the provisions of this invention and in accordance with the new method.

Figure 2 is a view of that portion of the transfer that has been applied to the surface of an object.

Figure 3 is an enlarged broken vertical section on the line indicated by 3-3, Fig. 1, the thickness of the various elements being exaggerated.

Figure 4 is a view similar to Fig. 3, showing two of the elements in reverse order to the showing in Fig. 3.

Ordinary transfers or decalcomanias are produced by printing with suitable ink upon specially prepared paper so that, when the paper is laid upon a smooth surface and dampened, said paper can be removed, leaving the printed matter upon said surface. Such transfers are not practical for use in the marking of packages that are exposed to the weather and subjected to friction in handling, as printer's ink soon becomes more or less obliterated, and one of the principal objects of this invention is to provide a type of transfer which is not open to the foregoing objections.

To make the transfers according to the principles of this invention, a stencil or stencils are made on bolting cloth, as is well understood in the art relating to the reproduction of colored designs by the use of cloth screens or stencils. One method of making said stencils is described in detail in my copending application Serial No. 119,040 filed June 28, 1926.

If the transfer is to be of the reverse type, as illustrated in Figs. 1 and 3, or, in other words, of the type which is necessary to be inverted when transferring to the surface on which the design is to appear, and if any of the design is to appear in ink, suitable decalcomania paper is first printed in the usual manner on a printing press to produce

a desired portion of the design as an ink coat on said paper. This ink coat is the first on the transfer but will be the last or undermost on the surface on which the design is to ultimately appear. Preferably, however, the ink employed is of considerably greater body or consistency than that usually used. The printing is done on the prepared side of the decalcomania paper, the coating of said prepared side containing an adhesive material, such as is known to the trade as dextrine.

The printed paper is then placed with the ink coat side uppermost beneath one of the cloth stencils mentioned above, and paint is forced through said stencil on top of the ink coat or impression. If more than one color of paint is to be applied, either a stencil for each color run will be used or the same stencil may be employed repeatedly by dissolving or otherwise removing a portion of the blocked area from the stencil after each color run. The making of a plurality of color runs either by the use of a single stencil or by the use of a plurality of stencils is well understood in the art relating to cloth stencil reproductions and, therefore, it is unnecessary to describe in detail herein how the preparation of these stencils is accomplished.

The paint that is to form the last coat of the transfer is specially prepared as there is mixed with said paint a special varnish, which may be made as follows: Take 100 pounds of the best grade of lime rosin and heat it to 450° F. Then sprinkle in the heated rosin, 5 pounds of litharge, maintaining the heat at 450° F. for one hour or until the rosin and litharge are combined. Then add 14 gallons of heavy bodied linseed oil and raise the temperature of the mixture to 500° F., and hold at this temperature for one hour, or until the mixture strings from a paddle upon cooling. Finally cool to 350° F. and carefully add 35 gallons of mineral turps, a little at a time.

The varnish above described, when dampened, becomes tacky or sticky. It is to be understood that any other suitable varnish that, when dampened with water, is sticky, can be used in place of that described. Of course, each of the successively applied coats of paint will be permitted to dry before the next succeeding coat is added.

According to the method described above,

I now have a transfer embodying a printed coat and superposed thereon one or more paint coats or, if desired, the ink coat may be omitted so that the transfer embodies merely superposed paint coats.

If the decalcomania paper comprises a base sheet and a tissue sheet on which the paint has been laid, said tissue sheet will first be pulled from the base sheet in a manner well understood in the art relating to such paper, as illustrated in Fig. 2.

To use this form of transfer, the surface to which it is to be applied will be cleaned with water and, while said surface is damp, the paint side will be placed on the damp surface, thus causing the varnish in the last applied or undermost coat of paint to become tacky or sticky. A wet sponge will be applied to the back of the transfer to dissolve the coating on the paper and said paper will then be pulled off, leaving the design in a series of superposed paint or paint and ink coats on the article to which it has been applied. Any surplus adhesive material that has come off of the decalcomania paper with the paint may be washed off and the paint will then remain an indefinite length of time.

If the transfer is of the slip-off type, as illustrated in Fig. 4, or, in other words, of a type in which the paper is slipped from between the paint coats and the surface on which the paint coats are to be applied, the operations described above of applying the ink and paint coats will be reversed so that the ink coat will be uppermost or the last applied and, furthermore, so that the paint having therein the varnish will constitute the lowermost coat or first applied.

To apply this slip-off type of transfer, the side of the paper not provided with paint will be applied to the damp surface and, after the paper has remained a sufficient length of time to dissolve the prepared surface having thereon the ink and paint coats, the operator will place his finger on the design of the transfer and grasp one

edge or corner of the paper and slip the same from beneath the paint coats so as to leave the paint coats upon the article to which said coats are to be applied.

It is to be understood that if the paint is to be applied to the decalcomania paper to produce a reverse type of transfer, as in Figs. 1 and 3, the stencils will be placed bottom face up on the paper so as to reverse the design on the paper in order that, when the design is applied to the surface that is to receive it, the design will appear unreversed, as illustrated in Fig. 2.

I claim:

1. The method of making transfers which consists in mixing together paint and a varnish that is sticky after it is dried and then dampened with water, and forcing the mixture thus made through a cloth stencil onto the prepared side of decalcomania paper.

2. The method of making transfers which consists in printing with heavy printer's ink upon the prepared side of decalcomania paper a portion of the design to be reproduced, drying said ink, mixing together paint and a varnish that is sticky after it is dried and then dampened with water, and forcing the mixture thus made through a cloth stencil having thereon another portion of the design and onto the decalcomania paper and at least partly overlying the printed portion.

3. A transfer comprising decalcomania paper, and a design thereon having a coat of paint as a part thereof, the paint coat having in it a varnish that is sticky when said coat is dampened with water.

4. A transfer comprising decalcomania paper, and a design thereon having a printed coat and a paint coat, the paint coat having in it a varnish that is sticky when said coat is dampened with water.

Signed at Los Angeles, California, this 19 day of June, 1926.

ROGER TULL.